

## 1

3,065,178

## LUBRICATING OIL COMPOSITION

Roland C. Nunn, Orinda, Calif., and Harold Martin Brewster, Linden, N.J., assignors to Esso Research and Engineering Company, a corporation of Delaware  
No Drawing. Filed Dec. 21, 1959, Ser. No. 860,634  
1 Claim. (Cl. 252—33.4)

This invention relates to an improved lubricating oil. More, particularly, the present invention relates to a lubricating oil composition of improved stability which comprises a major proportion of a lubricating oil, and synergistic amounts of a compound selected from the group consisting of orthoalkylated phenols and phenyl-alpha-naphthylamines in combination with highly basic magnesium sulfonates.

It has now been found and this finding forms the basis of the present invention, that the use of highly basic magnesium sulfonates in combination with an orthoalkylated phenol or a phenyl-alpha-naphthylamine in lubricating oils imparts surprising and unexpectedly improved oxidation stability to the lubricating oil fraction.

The lubricating oil compositions of the present invention are extremely useful as lubricants for internal combustion engines because of their outstanding oxidation stability at high temperatures. While the lubricants of this invention may be used to lubricate any type of internal combustion engine they are particularly important as crankcase lubricants for railway diesel locomotives since this particular type of diesel engine is designed to operate at rather high temperatures, especially under high load conditions.

The lubricating oil fraction employed in the practice of the present invention will preferably be a mineral lubricating oil of coastal or Mid-Continent origin. For example, the mineral lubricating oil base stock may be derived from Gulf Coastal, Panhandle, Pennsylvania, or California type crude oil. The lubricating oil fraction will preferably have a viscosity index in the range of 50-100 and a viscosity at 100° F. in the range of 800-1200 SSU. While the lubricating oil fraction is preferably a mineral lubricating oil, other lubricating oils may be employed in the composition of the present invention. Thus, lubricating oils produced synthetically by polymerizing olefins and/or esters to oils of the proper molecular weight and having the lubricating oil characteristics and viscosity ranges indicated may be used.

## 2

and 2,4,6 tri-tertiary butyl phenol. The alkyl groups of the orthoalkylated phenol will preferably contain about 1 to 6 carbon atoms. The 4,4'-methylene bis-(2,6 di-tertiary butyl phenol) is particularly preferred in the preparation of the lubricating oil compositions of this invention.

Phenyl-alpha-naphthylamine is well known in the prior art and has been used in various lubricating oil compositions as an anti-oxidant. Phenyl-alpha-naphthylamine and its preparation are disclosed in U.S. Patent 1,988,299.

The magnesium sulfonates useful in the present invention will be highly basic and have a total base number in the range of 100 to 400. The total base number is abbreviated TBN and is determined by standard potentiometric methods in accordance with ASTM D-664 test procedure. These highly basic magnesium sulfonates are available commercially and are known as Bryton 7560-B, 9076-A, 9199-A, 9200-A, etc. This type of highly basic magnesium sulfonate is normally prepared by treating a conventional magnesium sulfonate with magnesia and carbon dioxide.

The finished lubricating oil composition will contain in the range of 80 to 98 vol. percent of the lubricating oil fraction, 2 to 20 vol. percent of the highly basic magnesium sulfonate and 0.2 to 1.0 wt. percent, based on the total weight of the above composition, of an orthoalkylated phenol or phenyl-alpha-naphthylamine.

Other additives such as polymeric viscosity index improvers, pour point depressants, and anti-foaming amounts of silicone fluids may be added if desired.

## EXAMPLE I

In order to further illustrate the present invention, a number of compositions were made up in accordance with the present invention in which synergistic amounts of the orthoalkylated phenol and phenyl-alpha-naphthylamines were combined with the highly basic magnesium sulfonates. These compositions were compared with other compositions employing the orthoalkylated phenol and phenyl-alpha-naphthylamine in combination with various alkaline earth metal sulfonates.

Table I illustrates the various sulfonates, A through E, used in the preparation of the lubricating oil compositions of this invention and the sulfonates, F through I, used in the comparative formulations. The highly basic magnesium sulfonates of this invention were purchased from Bryton and the highly basic calcium sulfonates were purchased from Lubrizol Corp.

Table I  
RAILROAD DIESEL LUBRICANTS—HIGH ALKALINITY SULFONATES

|                         | Type                            | Over-based <sup>1</sup> with | TBN <sup>2</sup> | Percent CO <sub>3</sub> | Percent Ash <sup>3</sup> | Percent Ca | Percent Mg |
|-------------------------|---------------------------------|------------------------------|------------------|-------------------------|--------------------------|------------|------------|
| Sulfonate of invention: |                                 |                              |                  |                         |                          |            |            |
| A                       | Mg sulfonate <sup>4</sup> (30%) | Mg                           | 375              | 14.4                    | 44                       | —          | 8.9        |
| B                       | Mg sulfonate <sup>4</sup> (30%) | Mg                           | 115              | 4.25                    | —                        | —          | 3.52       |
| C                       | Mg sulfonate <sup>4</sup> (30%) | Mg                           | 178              | 5.12                    | 13.3                     | —          | 4.64       |
| D                       | Mg sulfonate <sup>4</sup> (30%) | Mg                           | 260              | 8.77                    | 17.6                     | —          | 6.36       |
| E                       | Mg sulfonate <sup>4</sup> (30%) | Mg                           | 300              | —                       | —                        | —          | —          |
| Comparative sulfonates: |                                 |                              |                  |                         |                          |            |            |
| F                       | Ca sulfonate (45%)              | Ca                           | 29               | —                       | 10.4                     | 2.9        | —          |
| G                       | Ca sulfonate (45%)              | Ca                           | 127              | 6.2                     | 21.5                     | 6.2        | —          |
| H                       | Ca sulfonate <sup>5</sup> (45%) | Mg                           | 75               | 3.3                     | 14                       | 1.7        | —          |
| I                       | Ca sulfonate <sup>5</sup> (45%) | Ca                           | 275              | —                       | —                        | —          | 1.7        |

<sup>1</sup> By adding excess Ca or Mg oxide and treating with CO<sub>2</sub>.

<sup>2</sup> Total base number (ASTM D-664).

<sup>3</sup> Sulfated.

<sup>4</sup> These Ca and Mg sulfonates were purchased from Bryton.

<sup>5</sup> This Ca sulfonate was purchased from Lubrizol Corp. as Lubrizol 56.

The orthoalkylated phenol is preferably an orthoalkylated phenol such as 2,6 di-tertiary-butyl phenol, 2,6 di-tertiary-2-dimethylamine para-cresol, 4,4'-methylene bis-(2,6 di-tertiary butyl phenol), ortho-tertiary butyl phenol,

70 Table II shows the actual formulation and results obtained in the E.R.E. stability test as well as the wear characteristics obtained in the three disc silver wear test for the lubricating oil formulations containing the magnesium

sulfonate-phenol combination of this invention. Table II also illustrates the improved results obtained with magnesium sulfonates over both neutral and high alkalinity calcium sulfonates.

The several blends were subjected to an E.R.E. stability test which comprises heating the lubricant to 340° F. in the presence of a Cu-Pb bearing and a silver strip and measuring the viscosity increase in terms of Saybolt seconds Universal after 19 and 23 hours. This test is used

Large increases in torque indicate severe wear while small increases in the torque readings indicate slight wear.

All the lubricants of this invention and the comparative formulations were prepared with a hydrofined, phenol extracted coastal distillate (boiling between 340° and 700° F. at 10 mm. mercury pressure), having a viscosity index of 63, as the lubricating oil fraction. The formulations were prepared by simple admixture of the additives with the above lubricating oil base.

Table II  
OXIDATION STABILITY AND SILVER LUBRICITY

| Type <sup>3</sup>        | Lubricant composition <sup>1</sup> |                                            | Vis.<br>SSU<br>at 100°<br>F. | E.R.E. stability test         |                                            |         |         | Three disc<br>silver wear<br>test rating |  |
|--------------------------|------------------------------------|--------------------------------------------|------------------------------|-------------------------------|--------------------------------------------|---------|---------|------------------------------------------|--|
|                          | Sulfonate                          | Phenol <sup>2</sup> ,<br>weight<br>percent |                              | Vis. inc. SSU/<br>100° F. at— | Cu-Pb bearing<br>weight loss in<br>mg. at— |         |         |                                          |  |
|                          | Vol.<br>percent                    |                                            |                              | 19 hrs.                       | 23 hrs.                                    | 19 hrs. | 23 hrs. |                                          |  |
| Lubricants of invention: |                                    |                                            |                              |                               |                                            |         |         |                                          |  |
| 1                        | A                                  | 5.0                                        | 0.8                          | 1,224                         | 39                                         | 50      | 0       | 1 Good-fair.                             |  |
| 2                        | A                                  | 10.0                                       | 0.8                          | 931                           | 26                                         | 33      | 0       | 1 Good.                                  |  |
| 3                        | A                                  | 5.0                                        | 0.2                          | 1,004                         | 34                                         | 55      | 3       | 8                                        |  |
| 4                        | A                                  | 10.0                                       | 0.2                          | 1,004                         | 26                                         | 38      | 1       | 2                                        |  |
| 5                        | B                                  | 5.0                                        | 0.8                          | 24                            | 55                                         | 2       | 4       | Fair.                                    |  |
| 6                        | B                                  | 10.0                                       | 0.8                          | 28                            | 62                                         | 2       | 4       | Do.                                      |  |
| 7                        | B                                  | 15.0                                       | 0.8                          | 46                            | 89                                         | 4       | 6       | Do.                                      |  |
| 8                        | C                                  | 5.0                                        | 0.8                          | 20                            | 24                                         | 0       | 0       | Good.                                    |  |
| 9                        | C                                  | 10.0                                       | 0.8                          | 36                            | 44                                         | 0       | 0       | Do.                                      |  |
| 10                       | C                                  | 15.0                                       | 0.8                          | 30                            | 39                                         | 0       | 0       | 0                                        |  |
| 11                       | D                                  | 5.0                                        | 0.8                          | 28                            | 33                                         | 0       | 1       | Fair.                                    |  |
| 12                       | D                                  | 10.0                                       | 0.8                          | 20                            | 25                                         | 0       | 0       | Good.                                    |  |
| 13                       | D                                  | 15.0                                       | 0.8                          | 21                            | 26                                         | 0       | 0       | Fair-poor.                               |  |
| Comparative lubricants:  |                                    |                                            |                              |                               |                                            |         |         |                                          |  |
| 14                       | F                                  | 5.0                                        | 0.8                          | 75                            | 260                                        | 31      | 127     | Excellent.                               |  |
| 15                       | G                                  | 5.0                                        | 0.8                          | 1,170                         | 352                                        | 993     | 9       | Poor.                                    |  |
| 16                       | G                                  | 10.0                                       | 0.8                          | 1,177                         | 97                                         | 298     | 5       | Very poor.                               |  |
| 17                       | H                                  | 5.0                                        | 0.8                          | 1,172                         | 520                                        | 839     | 145     | Good.                                    |  |
| 18                       | H                                  | 10.0                                       | 0.8                          | 1,189                         | 473                                        | 947     | 71      | Poor.                                    |  |
| 19                       | I                                  | 10.0                                       | 0.8                          | 929                           | 51                                         | 194     | 0       | Good.                                    |  |

<sup>1</sup> Base stock—63 VI undewaxed, severely hydrofined and phenol extracted coastal distillate.

<sup>2</sup> The phenol is 4,4'-methylene bis-(2,6 di-tertiary butyl phenol).

<sup>3</sup> Relates to designation given in Table I above.

to determine the stability of the lubricant to oxidation as shown by the viscosity increase as well as the lubricant's corrosiveness to silver-steel and copper-lead bearings.

The three disc silver wear test is a laboratory test developed to measure the silver wear prevention characteristics of railroad diesel lubricants when silver is used as a bear-

Table III shows the synergistic oxidation stability obtained by the combination of sulfonates with an orthoalkylated phenol and particularly the unexpected improvement in oxidation stability obtained when the sulfonate is a highly basic magnesium sulfonate, as illustrated by lubricants 28 through 30.

Table III

| Lubricant | Lubricant composition <sup>1</sup> |                                            | Vis. SSU<br>at 100° F. | E.R.E. lubricating stability<br>test (23 hrs. at 340° F.) |                                           |                                 |     | Three disc<br>silver wear<br>test rating |
|-----------|------------------------------------|--------------------------------------------|------------------------|-----------------------------------------------------------|-------------------------------------------|---------------------------------|-----|------------------------------------------|
|           | Sulfonate                          | Phenol <sup>2</sup> ,<br>weight<br>percent |                        | Vis. inc.<br>SSU at<br>100° F.                            | Cu-Pb<br>bearing<br>weight<br>loss in mg. | Silver<br>weight<br>loss in mg. |     |                                          |
|           | Type <sup>3</sup>                  | Vol.<br>percent                            |                        | 1,611                                                     | 313                                       | 156                             |     |                                          |
| 20        | A                                  | 5.0                                        | 0.0                    | 920                                                       | 1,004                                     | 189                             | 0.5 | Good.                                    |
| 21        | A                                  | 7.5                                        | 0.0                    | 955                                                       | 1,371                                     | 200                             | 0.5 | Do.                                      |
| 22        | A                                  | 10.0                                       | 0.0                    | 995                                                       | 1,066                                     | 110                             | 0.6 | Do.                                      |
| 23        |                                    | 0.0                                        | 0.8                    | 1,611                                                     | 313                                       | 156                             | 1.5 | Do.                                      |
| 24        |                                    | 0.0                                        | 0.25                   | 709                                                       | 313                                       | 144                             | 3.9 |                                          |
| 25        | A                                  | 5.0                                        | 0.2                    | 931                                                       | 55                                        | 8                               | 0.2 |                                          |
| 26        | A                                  | 7.5                                        | 0.2                    | 965                                                       | 73                                        | 1                               | 0.4 |                                          |
| 27        | A                                  | 10.0                                       | 0.2                    | 1,004                                                     | 36                                        | 2                               |     |                                          |

<sup>1</sup> Base stock—63 VI undewaxed, severely hydrofined and phenol extracted coastal distillate.

<sup>2</sup> The phenol is 4,4'-methylene bis-(2,6 di-tertiary butyl phenol).

<sup>3</sup> Relates to designation given in Table I above.

ing surface for steel. The results obtained in this test are important since about 65% of all railway diesel engines use a silver-on-steel surfaced bearing. The test consists of rotating a steel ball at 600 r.p.m. on three stationary silver discs under a constantly applied load of 10 kg. in the presence of the test lubricant at 150° C. Torque is measured after one minute of operation and every two minutes thereafter, up to a total test time of 15 minutes.

Table IV illustrates the overall performance in a Chevrolet L-4 engine test of a lubricating oil composition of this invention as compared with similar experimental and commercial lubricating oil compositions. Lubricant "32" of Table IV is representative of the lubricating oil compositions of this invention while lubricants 33, 34 and 35 represent comparative compositions.

The Chevrolet L-4 engine test is well known in the

art and uses a standard 6-cylinder Chevrolet engine fitted with copper-lead bearings. Here the engine was run con-

obtained in Table III for the phenol-magnesium sulfonates of this invention.

Table V

| Base Stock <sup>1</sup> plus              |                                                              | Viscosity<br>SSU at<br>100° F. | ERE lubricant stability test              |         |                                              |                                               |  |
|-------------------------------------------|--------------------------------------------------------------|--------------------------------|-------------------------------------------|---------|----------------------------------------------|-----------------------------------------------|--|
| Mg sulfo-<br>nate, vol.<br>percent        | Phenyl-<br>alpha-<br>naph-<br>thyamine,<br>weight<br>percent |                                | Viscosity Increase,<br>SSU at 100° F. at— |         | Bearing<br>weight<br>loss at 23<br>hrs., mg. | Silver<br>weight<br>change at 23<br>hrs., mg. |  |
|                                           |                                                              |                                | 19 hrs.                                   | 23 hrs. |                                              |                                               |  |
| 0.0                                       | 0.5                                                          | 621                            | 525                                       | 800     | 279                                          | -1.6                                          |  |
| <sup>2</sup> 5.0                          | 0.0                                                          | 920                            | 765                                       | 1,004   | 189                                          | -0.5                                          |  |
| <sup>2</sup> 10.0                         | 0.0                                                          | 995                            | 769                                       | 1,066   | 110                                          | -0.6                                          |  |
| <sup>3</sup> 5.0                          | 0.4                                                          | 917                            | 73                                        | 88      | 6                                            | 0.0                                           |  |
| <sup>3</sup> 10.0                         | 0.4                                                          | 933                            | 63                                        | 74      | 1                                            | 0.0                                           |  |
| <sup>3</sup> 15.0                         | 0.4                                                          | 946                            | 71                                        | 84      | 0                                            | -0.1                                          |  |
| Ca sulfonate <sup>4</sup><br>vol. percent |                                                              |                                |                                           |         |                                              |                                               |  |
| 10.0                                      | 0.4                                                          | 901                            | 800                                       | 1,103   | 67                                           | 0.0                                           |  |

<sup>1</sup> 63 V.I. undewaxed, severely hydrofined and phenol extracted coastal distillate having a viscosity at 210° F. of 60-80 SSU.

<sup>2</sup> TBN (D-664)=375.

<sup>3</sup> TBN (D-664)=300.

<sup>4</sup> TBN (D-664)=275 (purchased as Lubrizol 56).

tinuously for 36 hours after which time the piston deposits and weight loss of the Cu-Pb bearings were measured and an inspection of the used lubricant was made. The Chevrolet L-4 engine test is important since it gives a good indication of the oil's oxidation stability under actual operating conditions.

Table IV  
CHEVROLET L-4 EVALUATION

| Lubricant       | Cu-Pb <sup>1</sup><br>BWL, mg. | Piston deposit <sup>2</sup> merit<br>rating |                 | Vis. inc.<br>SSU/<br>100° F. |
|-----------------|--------------------------------|---------------------------------------------|-----------------|------------------------------|
|                 |                                | Overall                                     | Piston<br>skirt |                              |
| 32 <sup>3</sup> | 60                             | 97.3                                        | 96.6            | 9                            |
| 33 <sup>4</sup> | 120                            | 96.5                                        | 93.9            | 197                          |
| 34 <sup>5</sup> | 22                             | 97.3                                        | 97.7            | 85                           |

<sup>1</sup> Represents the weight loss in mg. of the copper-lead bearing.

<sup>2</sup> Represents piston cleanliness based on visual rating of 0 to 100, 0 being completely covered with deposits and 100 being completely free of deposits.

<sup>3</sup> Same as lubricant 2 of Table II.

<sup>4</sup> 93.75 vol. percent of base stock of Table II, 2.25 vol. percent of Ca-Ba nyl phenol sulfide, 4.0 vol. percent of sulfonate F of Table I and 0.4 weight percent phenyl-alpha-naphthylamine.

<sup>5</sup> 95.0 vol. percent of same base stock of Table II but 5.0 vol. percent of sulfonate F of Table I and 0.8 weight percent of 4,4'-methylene bis(2,6 di-tertiary butyl phenol).

The fact that synergistically improved oxidation stability can be obtained by combining the highly basic magnesium sulfonates of this invention with phenyl-alpha-naphthylamine is shown in the following table. The improved oxidation stability obtained with the phenyl-alpha-naphthylamine-magnesium sulfonate combination is comparable with the unexpected and surprising improvement

In summary, Table I characterizes the highly basic magnesium sulfonates of this invention. Tables II through IV illustrate the surprising oxidation stability and wear resistance obtained by the combination of these highly basic magnesium sulfonates with an orthoalkylated phenol in a lubricating oil fraction. Table V shows that phenol-alpha-naphthylamine will also impart an unexpectedly high oxidation stability to the lubricating oil fraction when combined with the highly basic magnesium sulfonates of this invention.

Tables II and V are of particular importance since they show advantage for magnesium sulfonates over calcium sulfonates in the same base number range. They also show that a total base number in the range of 100 to 400 and preferably in the range of about 150 to 300 is preferred.

What is claimed is:

A lubricating oil composition consisting essentially of a hydrofined and phenol extracted mineral lubricating oil having a viscosity index of about 50 to about 100, and a synergistic combination with regard to oxidation inhibition of about 5 to 10 volume percent of a 30 wt. percent concentrate in mineral oil of a high basic magnesium sulfonate having a total base number about 375, and about 0.2 wt. percent of 4,4'-methylene bis-(2,6 di-tertiary butyl phenol).

#### References Cited in the file of this patent

#### UNITED STATES PATENTS

- 55 2,629,693 Barton et al. ----- Feb. 24, 1953  
2,695,273 Hook et al. ----- Nov. 23, 1954  
2,807,653 Filbey et al. ----- Sept. 24, 1957  
2,856,359 Schlicht ----- Oct. 14, 1958  
60 2,895,913 Carlyle et al. ----- July 21, 1959

#### FOREIGN PATENTS

- 454,227 Canada ----- Jan. 18, 1949